

## UNITED STATES PATENT OFFICE

2,506,059

## WAX COMPOSITIONS

John R. Bowman and William P. Ridenour, Pittsburgh, Pa., assignors to Gulf Research & Development Company, Pittsburgh, Pa., a corporation of Delaware

No Drawing. Application June 7, 1946,  
Serial No. 675,318

5 Claims. (Cl. 106—268)

1

This invention relates to improved wax compositions and more particularly to paraffin wax compositions containing an additive to increase the tensile strength thereof.

Paraffin wax and paraffin wax products are used in many industries. In many of its applications and particularly in coating paper for such uses as wrapping, it is desirable to have as high a tensile strength as possible while at the same time retaining all of the desirable characteristics of a substantially pure paraffin wax. These other desirable characteristics include a high melting point, a uniform crystalline structure, and freedom from scuffing and mottling.

An object of the present invention is to provide paraffin wax compositions with increased tensile strength.

A further object of the invention is to provide an improved paraffin wax composition with increased tensile strength while at the same time retaining the other desirable features of paraffin wax.

These and other objects of this invention are achieved by a composition comprising paraffin wax and from about 0.1 per cent to about 0.5 per cent by weight of a wax-soluble aluminum soap.

The method for obtaining the improved wax comprises thoroughly mixing paraffin wax in a molten state with the aluminum soap.

Of the aluminum soaps useful in the invention, aluminum stearate is preferable. Aluminum soaps of other fatty acids may be used so long as they are wax-soluble. These include the saturated fatty acid soaps in the range above C<sub>12</sub>.

The amount of the aluminum soap to be added may be varied, between about 0.1 per cent and about 0.5 per cent; 0.5 per cent is preferable. While amounts varying slightly from either of these limits may give some desirable results, amounts substantially larger than 0.5 per cent

are undesirable. For example, at 0.75 per cent aluminum stearate in paraffin wax does not form a true solution, but by vigorous stirring a colloidal suspension may be obtained. Distinct plastic properties are evident and on brief standing a gel is formed which on re-stirring breaks up to give a distinctly non-homogeneous mixture.

The aluminum stearate used in the composition should be the di- or tri-stearate, the mono-stearate showing no improvement as it is practically insoluble in the paraffin wax. The aluminum di- or tri-stearate may be any of the products commercially available, but as will be seen from the test data below, that which is free of fatty acid is most desirable. It may be necessary to treat the commercial aluminum stearates by washing with a fatty acid solvent such as absolute ethyl alcohol, acetone, ethylacetate, etc. to remove the free acid.

The various types of paraffin wax may be improved according to the present invention, but the invention is particularly applicable to the grades of paraffin wax low in oil content. Improvement has been noted in a refined 122° F. ASTM melting point paraffin wax, but the highest tensile strength has been obtained with a highly refined paraffin wax having an ASTM melting point of 132° F.

The wax composition may contain other ingredients than paraffin and aluminum soaps but it will be understood that these ingredients should not be of a type or quantity that will substantially reduce the tensile strength, such as for example, oil.

The table below illustrates the tensile strength results obtained with a highly refined paraffin wax having an ASTM melting point of 132° F. The aluminum stearate used had the free fatty-acid content indicated in the table and the acid-free samples were obtained by washing with ethyl alcohol.

TABLE

Blends of aluminum stearate and paraffin wax  
(132° F. E. M. P.)

|          | Per cent<br>Added | Free Fatty<br>content of<br>soap, per cent | Tensile<br>strength 70°<br>F. Lbs. pull | Lbs. im-<br>provement of<br>blend over<br>straight wax | Lbs. im-<br>provement of<br>acid-free over<br>commercial<br>stearate |
|----------|-------------------|--------------------------------------------|-----------------------------------------|--------------------------------------------------------|----------------------------------------------------------------------|
| Di.....  | 0.0               | 4.59                                       | 93±1.5                                  | 0                                                      | -----                                                                |
| Di.....  | 0.1               | 4.59                                       | 101±1.5                                 | 8                                                      | -----                                                                |
| Di.....  | 0.5               | 4.59                                       | 126±1.0                                 | 33                                                     | -----                                                                |
| Di.....  | 0.0               | 0.0                                        | 98±2.0                                  | 0                                                      | -----                                                                |
| Di.....  | 0.5               | 0.0                                        | 136.2±3.8                               | 38                                                     | +5                                                                   |
| Tri..... | 0.0               | 17.77                                      | 93±1.5                                  | 0                                                      | -----                                                                |
| Tri..... | 0.1               | 17.77                                      | 97±1.5                                  | 4                                                      | -----                                                                |
| Tri..... | 0.5               | 17.77                                      | 123±6.0                                 | 30                                                     | -----                                                                |
| Tri..... | 0.0               | 0.0                                        | 98±2                                    | 0                                                      | -----                                                                |
| Tri..... | 0.25              | 0.0                                        | 130±2.5                                 | 32                                                     | +19                                                                  |
| Tri..... | 0.50              | 0.0                                        | 146±1.9                                 | 48                                                     | +18                                                                  |

It will be seen from the above table that the commercial di-stearate is more effective than the tri-stearate, but this is apparently for the reason that the free acid content of the tri-stearate is substantially higher. On removal of the free acid, the tri-stearate becomes the more effective additive.

The preferable composition is a highly refined paraffin wax containing about 0.5 per cent of aluminum tri-stearate substantially free of acid.

Free fatty acids not only reduce the tensile strength of the wax, but tend to cause the wax to crumble, increase scuffing and cause mottling. These effects oppose the desirable ones induced by aluminum soaps; therefore aluminum soaps as low as possible in free fatty acid contents are desirable. However, commercial aluminum soaps which contain free fatty acids in the ordinary amounts are tolerable.

The addition of the above specified amount of the aluminum soap to the paraffin wax increases the tensile strength and reduces mottling, as set forth above. In addition, opacity is considerably increased as is also ductility. Paraffin waxes containing aluminum soaps will stand considerably greater stretching and bending before breaking than paraffin waxes without the aluminum soap. The texture of the wax surface is slightly altered, becoming unctuous or soapy to the touch and having less tendency to scuff under mild abrasion.

What we claim is:

1. A solid paraffin wax composition of increased tensile strength consisting essentially of paraffin wax and from about 0.1 per cent to about 0.5 per cent of aluminum stearate wherein there are at least two stearate radicals per aluminum atom and said aluminum stearate is substantially free of acid.

2. A solid paraffin wax composition of increased tensile strength consisting essentially of refined paraffin wax and about 0.5 per cent of

aluminum tri-stearate substantially free of acid.

3. A solid paraffin wax composition of increased tensile strength consisting essentially of refined paraffin wax having a melting point of about 132° F. and about 0.5 per cent of aluminum tri-stearate substantially free of acid.

4. A method for making a composition consisting essentially of solid paraffin wax of increased tensile strength comprising washing a commercial aluminum tri-stearate with ethyl alcohol until it is substantially acid-free and mixing it with molten paraffin wax in proportion such that the wax contains from about 0.1 per cent to about 0.5 per cent of said aluminum tri-stearate.

5. A method for making a composition consisting essentially of solid paraffin wax of increased tensile strength comprising washing a commercial aluminum stearate wherein there are at least two stearate radicals for each aluminum atom with a solvent until it is substantially acid-free and mixing it with molten paraffin wax in proportion such that the wax contains from about 0.1 per cent to about 0.5 per cent of said aluminum stearate.

JOHN R. BOWMAN.

WILLIAM P. RIDENOUR.

#### REFERENCES CITED

The following references are of record in the file of this patent:

#### UNITED STATES PATENTS

| Number    | Name           | Date           |
|-----------|----------------|----------------|
| 2,130,560 | Plechner       | Sept. 20, 1938 |
| 3,320,644 | Nill           | June 1, 1943   |
| 2,359,946 | Sudholz et al. | Oct. 10, 1944  |

#### OTHER REFERENCES

Metallic Soaps, published by Metasap Chemical Co. (1940), p. 26.